

3,788,994  
**PRESSURE FIXABLE ELECTROSTATOGRAPHIC  
TONER**

Russel E. Wellman, Pittsford, and Richard G. Crystal,  
Penfield, N.Y., assignors to Xerox Corporation, Stam-  
ford, Conn.

No Drawing. Filed Dec. 30, 1971, Ser. No. 214,374  
Int. Cl. G03g 9/00

U.S. Cl. 252—62.1

9 Claims

#### ABSTRACT OF THE DISCLOSURE

Pressure and heat/pressure fixable encapsulated electro-  
statalographic toners comprising adhesive, soft-solid core  
materials encapsulated in a polymeric shell material. De-  
veloper compositions employing the encapsulated toners  
and methods of forming visible electrostatographic toner  
images are also disclosed.

#### BACKGROUND OF THE INVENTION

This invention relates to electrostatography, and more  
particularly, to improved electrostatographic developing  
materials and the use thereof.

The formation and development of images on the sur-  
face of photoconductive materials by electrostatographic  
means is well known. The basic electrostatographic pro-  
cess, as taught by C. F. Carlson in U.S. Pat. 2,297,691,  
involves placing a uniform electrostatic charge on a  
photoconductive insulating layer, exposing the layer to a  
light and shadow image to dissipate the charge on the  
areas of the layer exposed to the light and developing the  
resulting electrostatic latent image by depositing on the  
image a finely divided electroscopic material referred to  
in the art as "toner." The toner will normally be attracted  
to those areas of the layer which retain a charge, thereby  
forming a toner image corresponding to the electrostatic  
latent image. This powder image may then be transferred  
to a support surface such as paper. The transferred image  
may subsequently be permanently affixed to the support  
surface as by heat. In such case, the toner must generally  
be heated to a temperature at which the toner flows in  
order to effect fusing of the toner to the support medium.  
Instead of latent image formation by uniformly charging  
the photoconductive layer and then exposing the layer  
to a light and shadow image, one may form the latent  
image by directly charging the layer in image configura-  
tion. The powder image may be fixed to the photocon-  
ductive layer if elimination of the powder image transfer  
step is desired. Other suitable fixing means such as solvent  
or overcoating treatment may be substituted for the fore-  
going heat fixing steps.

Several methods are known for applying the electro-  
scopic particles to the electrostatic latent image to be  
developed. One development technique, as disclosed by  
E. N. Wise in U.S. Pat. 2,618,552, is known as "cascade"  
development. In this method, a developer material com-  
prising relatively large carrier particles having finely di-  
vided toner particles electrostatically coated thereon is  
conveyed to and rolled or cascaded across the electrostatic  
latent image bearing surface. The composition of the  
carrier particles is so selected as to triboelectrically charge  
the toner particles to the desired polarity. As the mixture  
cascades or rolls across the image bearing surface, the  
toner particles are electrostatically deposited and secured  
to the charged portion of the latent image and are not  
deposited on the discharged or background portions of  
the image. Most of the toner particles accidentally de-  
posited in the background are removed by the rolling  
carrier, due apparently to a greater electrostatic attraction  
between the toner and the carrier than between the toner  
and the discharged background. The carrier and excess

toner are then recycled. This technique is extremely good  
for the development of line copy images.

Another method of developing electrostatic images is  
the "magnetic brush" process as disclosed, for example,  
in U.S. Pat. 2,874,063. In this method, a developer ma-  
terial container toner and magnetic carrier particles are  
carried by a magnet. The magnetic field of the magnet  
causes alignment of the magnetic carrier into a brushlike  
configuration. This "magnetic brush" is engaged with the  
electrostatic image bearing surface and the toner particles  
are drawn from the brush to the latent image by electro-  
static attraction.

Still another technique for developing electrostatic  
latent images is the "powder cloud" process as disclosed,  
for example, by C. F. Carlson in U.S. Pat. 2,221,776.  
In this method, a developer material comprising electri-  
cally charged toner particles in a gaseous fluid is passed  
adjacent to the surface bearing the electrostatic latent  
image. The toner particles are drawn by electrostatic at-  
traction from the gas to the latent image. This process is  
particularly useful in continuous tone development.

Other development methods, such as "touchdown"  
development as disclosed by R. W. Gundlach in U.S. Pat.  
3,166,432 may be used where suitable.

Although some of the foregoing development tech-  
niques are employed commercially today, the most widely  
used commercial electrostatographic development tech-  
nique is the process known as "cascade" development.  
A general purpose office copying machine incorporating  
this development method is described in U.S. Pat. 3,099,-  
943. The cascade development technique is generally  
carried out in a commercial apparatus by cascading a de-  
veloper mixture over the upper surface of an electrostatic  
latent image bearing drum having a horizontal axis. The  
developer is transported from a trough or sump to the  
upper portion of the drum by means of an endless belt  
conveyor. After the developer is cascaded downward along  
the upper quadrant surface of the drum into the sump,  
it is recycled through the developing system to develop  
additional electrostatic latent images. Small quantities of  
toner are periodically added to the developing mixture to  
compensate for the toner depleted by development. The  
resulting toner image is usually transferred to a receiving  
sheet and thereafter fused by suitable means such as an  
oven. The surface of the drum is thereafter cleaned for  
reuse. This imaging process is then repeated for each  
copy produced by the machine and is ordinarily repeated  
many thousands of times during the usable life of the  
developer.

The toners employed in the art are generally fixed to  
a support medium by the application of heat and, there-  
fore, such toners must be heated to a temperature at which  
the toner flows in order to effect fusing of the toner to  
the support medium. The fusion technique, although high-  
ly successful, has some disadvantages; namely; such a

technique has not been readily adaptable to high speed  
machines as a result of the time or energy required  
to raise the temperature of the toner to a temperature  
at which the toner can be fused to the support medium.

Attempts to rapidly fuse a high melting point toner by  
means of oversized high capacity heating units have been  
confronted with the problems of preventing the charring  
of paper receiving sheets and of adequately dissipating  
the heat evolved from the fusing unit or units. Thus, in  
order to avoid charring or combustion, additional equip-  
ment such as complex and expensive cooling units are  
necessary to properly dispose of the large quantity of  
heat generated by the fuser. Incomplete removal of the  
heat evolved will result in operator discomfort and  
damage to heat sensitive machine components. Further,  
the increased space occupied by and the high operating

costs of the heating and cooling units often outweigh the advantages achieved by the increased machine speed. On the other hand, toners made from low melting, usually low molecular weight resins which are easily heat fused at relatively low temperatures are usually undesirable because these materials tend to form thick films on reusable photoconductor surfaces. These films tend to cause image degradation and contribute to machine maintenance down time. Many low molecular weight resins decompose when subjected to fusing conditions in high speed copying and duplicating machines. In addition, the low melting toners tend to form tacky images on the copy sheet which are easily smudged and often offset to other adjacent sheets. Further, the low melting toners become tacky at temperatures that may be encountered in storage or in the high speed machines. This usually causes "blocking" or caking of the toner or developer in storage and in the machine and poor or erratic dispensing prior to and during machine operation. Additionally, these materials are often extremely difficult or even impossible to comminute in conventional grinding apparatus because they become tacky at the temperatures attained during the grinding operation. Also, the toner material must be capable of accepting a charge of the correct polarity when brought into rubbing contact with the surface of carrier materials in cascade or touchdown development systems. The triboelectric and flow characteristics of many toners are adversely affected by changes in the ambient humidity. For example, the triboelectric values of some toners fluctuate with changes in relative humidity and are not desirable for employment in electrostatographic systems, particularly in precision automatic machines which require toners having stable and predictable triboelectric values. Another factor affecting the stability of carrier triboelectric properties is the tendency of some toner materials to "impact" on the surface of carrier particles. When developers are employed in automatic developing machines and recycled through many cycles, the many collisions which occur between the carrier and toner particles in the machine cause the toner particles carried on the surface of the carrier particles to be welded or otherwise forced into the surface of the carrier particles. The gradual accumulation of permanently attached toner material on the surface of carrier particles causes a change in the triboelectric value of the carrier particles and directly contributes to the degradation of copy quality by eventual destruction of the toner carrying capacity of the carrier. Numerous known carriers and toners are abrasive in nature. Abrasive contact between toner particles, carriers, and electrostatographic imaging surfaces accelerates mutual deterioration of these components. In addition, both filming of reusable photoconductor surfaces and impaction contribute to the phenomenon known as "bead sticking" which is the adherence of carrier beads to reusable photoconductor surfaces. When this occurs, the rubbing of the carrier beads across the photoconductor surface during cleaning operations leads to scratching and abrasion of the reusable photoconductor surface. Replacement of carriers and electrostatic image bearing surfaces is expensive and time consuming. Electrostatographic copies should possess good line image contrast as well as acceptable solid area coverage. However, when a process is designed to improve either line image contrast or solid area coverage, reduced quality of the other can be expected. Attempts to increase image density by depositing greater quantities of toner particles on the electrostatic latent image are usually rewarded with an undesirable increase in background deposits.

Another disadvantage of copying machines that utilize heat to fix the thermoplastic toner materials to the image support medium is that the machines generally do not function properly immediately after their idle hours. That is, it takes a certain amount of time until the temperature

of the heating system reaches the operating temperature. Therefore, it is usually necessary to maintain the temperature of the heating system at about its operating temperature in order that the machine can operate satisfactorily shortly after it is turned on. This obviously means that heat energy is constantly lost while the machine is idle.

The toner particles are usually thermoplastic resins selected to have melting points significantly above any ambient temperatures that might be encountered during electrostatic deposition. In addition to the developing powder or toner materials described in U.S. Pat. 2,297,691, a number of additional toner materials have been developed especially for use in the newer development techniques including the cascade technique described above. Generally speaking, these new toner materials have comprised various improved resins mixed with different pigments such as carbon black. Some exemplary patents along this line include U.S. Pat. 2,659,670 to Copley which describes a toner resin of rosin-modified phenol-formaldehyde, U.S. Re. 25,136 to Carlson which describes an electrostatographic toner employing a resin of polymerized styrene and U.S. Pat. 3,079,342 to Insalaco describing a plasticized copolymer resin in which the comonomers are styrene and a methacrylate selected from the group of butyl, isobutyl, ethyl, propyl, and isopropyl.

In the past, these toners have generally been prepared by thoroughly mixing a heat softened resin and colorant to form a uniform dispersion as by blending these ingredients in a rubber mill or the like and then pulverizing this material after cooling to form it into small particles. Although toners manufactured by this technique have resulted in some very excellent toner, they do tend to have certain shortcomings. For example, the toners generally have a rather wide range of particle sizes. That is, even though the average toner particle size made according to this technique generally ranges between about 5 and 10 microns, individual particles ranging from submicron in size to above 20 microns are not infrequently produced. In addition, toner produced by this technique imposes certain limitations upon the material selected for the toner because the colored resin must be sufficiently friable so that it can be pulverized at an economically feasible rate of production. The problem which arises from this requirement is that when the colored resin is sufficiently friable for really high speed pulverizing, it tends to form even a wider range of particle sizes during pulverization including relatively large percentages of fines and is frequently subject to even further pulverization or powdering when it is employed for developing in electrostatographic imaging apparatus. All other requirements of electrostatographic developers or toners including the requirements that they be stable in storage, nonagglomerative, have the proper triboelectric properties for developing and have a low melting point for heat fusing are only compounded by the additional requirements imposed by this toner forming process. Some developer materials such as those containing toner particles made from low molecular weight resins though possessing desirable properties such as proper triboelectric characteristics, are unsuitable because they tend to cake, bridge and agglomerate during handling and storage.

Of potential interest as electrostatographic developer materials are the pressure fixable toner materials because of their very low energy requirements. However, the toner requirements for good machine performance tend to be diametrically opposed to the requirements for pressure fixing. That is, low toner impaction requires a higher toner softening temperature and good mechanical strength while pressure fixing requires softening and viscous flow at room temperature. In addition, one of the problems with potential pressure fixable toners is the need to gently handle these materials prior to pressure fusion to paper or other suitable medium so that these materials

will not prefuse and cause impaction in the development chamber. A balance must generally be made between a material which will pressure fix onto paper at low pressure but yet not impact in the development chamber. A major cause of such prefusion is the abrasive action of the tumbling carrier beads on the toner both in normal cascade development and magnetic brush development.

The production of an encapsulated electrostatographic toner material which can be pressure fixed would be desirable and advantageous since unencapsulated materials which undergo cold flow tend to form tacky images on the copy sheet which often offset to other adjacent sheets. Toner particles containing unencapsulated materials which undergo cold flow tend to bridge, cake and block during production and in the shipping container as well as in the electrostatographic imaging machine. Also, the toner material should be capable of accepting a charge of the correct polarity such as when brought into rubbing contact with the surface of carrier materials in cascade, magnetic brush or touchdown development systems. Some toner materials which possess many properties which would be desirable in electrostatographic toners dispense poorly and cannot be used in automatic copying and duplicating machines. Other toners dispense well but form images which are characterized by low density, poor resolution, or high background. Further, some toners are unsuitable for processes where electrostatic transfer is employed.

A useful form of liquid phase separation from aqueous media is known as coacervation and is exemplified in U.S. Pats. 2,800,457 and 2,800,458 to Green. However, toner materials obtained by this method such as those comprising encapsulated inks are generally fragile, their shells are loose after fixing and tend to cause smearing of the developed image. In addition, such toner materials generally have poor electrostatographic properties since the encapsulated contents tend to diffuse through the shell material leading to alteration of triboelectric properties. Further, broken liquid core materials adversely affect copy quality due to vertical and lateral bleeding resulting in poor resolution. Other patents such as U.S. Pats. 3,080,250 and 3,386,822 disclose capsules containing solvents which tackify some portion of the toner and help to fix the image. However, such patented materials are encapsulated liquids and once the capsule is crushed, the contents will flow perceptively with little or no applied stress and because of the solvent, the presence of vapors is usually undesirable.

Since most toner materials are deficient in one or more of the above areas, there is a continuing need for improved toners and developers.

#### SUMMARY OF THE INVENTION

It is, therefore, an object of this invention to provide a developer overcoming the above noted deficiencies.

It is another object of this invention to provide a toner which is stable at toner fusing conditions in high speed copying and duplicating machines.

It is another object of this invention to provide impaction resistant toner materials.

It is another object of this invention to form a toner which can be fused at higher rates with less heat energy.

It is another object of this invention to provide a toner which is triboelectrically stable.

It is another object of this invention to provide a toner which is resistant to smearing.

It is another object of this invention to provide a toner which is resistant to agglomeration.

It is another object of this invention to provide a toner which is readily removable by carriers from background areas during image development.

It is another object of this invention to provide a toner which may be easily cleaned from electrostatic imaging surfaces.

It is another object of this invention to provide a toner which reduces mechanical abrasion of electrostatic imaging surfaces.

It is another object of this invention to provide a toner which is effective at low initial electrostatic surface potentials.

It is another object of this invention to provide a toner which forms dense toner images.

It is another object of this invention to provide a toner which is readily transferrable from an electrostatographic imaging surface to a transfer surface.

It is another object of this invention to provide a toner which is resistant to mechanical attrition during the development process.

It is another object of this invention to provide a toner which can be fused at higher rates with less pressure.

It is another object of this invention to provide an encapsulated toner containing a core material which will flow perceptively only under significant applied stress and have sufficient cohesive strength to form a good bond between the capsule shell and an image substrate.

It is another object of this invention to provide a toner and developer having physical and chemical properties superior to those of known toners and developers.

The above objects and others are accomplished by providing an electrostatographic toner comprising adhesive, soft-solid core materials encapsulated in a shell material. The pressure fixable toners of this invention include any encapsulated toner in which the core material is an adhesive soft-solid at ambient temperature or becomes an adhesive soft-solid when heated to a temperature between about 70° F. and about 250° F. The term adhesive soft-solid is intended to include any material showing no perceptible flow under slight stress in a short observation period, but showing significant flow under large applied stresses and which is capable of forming a strong adhesive bond. The encapsulated pressure fixable toners of this invention include electrostatographic encapsulated toners containing a cold flowable adhesive polymeric core material. Thus, core materials having a viscosity at a shear rate of about 75 sec.<sup>-1</sup> of between about  $5 \times 10^4$  and about  $10^8$  poise at ambient temperature and a glass transition temperature (Tg) below about 30° C. may be employed in the encapsulated toners of this invention which are pressure fixable without the assistance of heat. In addition, core materials having a viscosity at a shear rate of about 75 sec.<sup>-1</sup> of between about  $5 \times 10^4$  and about  $10^8$  poise at the temperature of a pressure fixing device and a glass transition temperature below or not more than a few degrees above the temperature of a pressure fixing device may be employed in the encapsulated toners of this invention. Thus, core materials having a higher glass transition temperature or a higher viscosity at ambient temperature may be used where the encapsulated toners of this invention are fixed using a combination of pressure and heat. For example, where a heat-assisted pressure fixing mode is employed in which one roll, typically a steel roll, is heated to about 45° C., core materials having a viscosity between about  $5 \times 10^4$  and about  $10^8$  poise at about 45° C. may be employed. Where the core material has more than one detectable glass transition temperature, such as when it contains two or more phases, only one glass transition temperature has to be below the temperature conditions given above. In some cases, it is advantageous to use core materials which are shear sensitive, that is, those which exhibit distinctly different viscosities depending on the effective shear rate. With shear sensitive core materials, the viscosity at very low shear rates may be much higher than the range given above. However, at the shear rate occurring in the pressure fixing device used, the viscosity should be below about  $10^8$  poise.

Any suitable pressure may be employed to fix the toners of this invention. Typical pressures are those below

about 600 p.l.i. since higher pressures tend to calender some paper substrates and change their texture and finish. In any event, the upper limit of usable pressure is a function of the substrate used. Any suitable temperature may be employed to fix the toners of this invention with a heat-assisted pressure fixing electrostatographic device. Typical temperatures in such a device include temperatures from about 100° F. to about 160° F.

Suitable shell materials generally have a viscosity higher than the core materials and usually are materials which will not flow at moderate pressures and temperatures likely to be encountered during storage. Thus, amorphous shell materials having a glass transition temperature above about 50° C. and crystalline shell materials having a melting point above about 40° C. may be employed in the encapsulated toners of this invention. Where the shell materials exhibit more than one glass transition temperature or melting point, they generally will have at least one glass transition temperature above about 50° C. or a melting point above about 40° C., and the other glass transition temperature or melting point may be above or below these temperatures. It is generally preferable for the shell materials to be brittle and somewhat friable because these properties permit facile and complete rupturing of the encapsulated toners to thereby release the adhesive core materials. However, for some applications, it is preferable to employ shell materials which are tough and less rigid under fixing conditions. That is, the shell material may exhibit slight flow under applied pressures at fixing temperatures. This type of shell materials is particularly useful when employing both heat and pressure for fixing the toner image. Suitable shell materials embrace a very wide range of rheological properties, since variations in the properties of the shell material can to a large extent be compensated for by adjustment of the shell thickness. In addition, the properties of suitable shell materials depend on the properties of the core material employed. Thus, the combination of the modulus of elasticity of the shell material and the shell thickness is adjusted to compensate for the viscosity of the core material used so that the shell will fracture if brittle, or rupture if ductile, under the fixing conditions of temperature and pressure employed. Thus, shell materials having a modulus of elasticity of above about 100 p.s.i. and a compressive strength of above about 500 p.s.i. provide satisfactory results. However, shell materials having a modulus of elasticity of above about 1000 p.s.i. and a compressive strength of above about 2000 p.s.i. are preferred because the resulting encapsulated toner particles provide enhanced fixing properties and freedom from impaction. Thus, shell materials such as polystyrenes, polycarbonates, and the reaction products of dimer acids with linear diamines are some of the preferred shell materials.

It has been found that there is a correlation between the glass transition temperature of the core material and the pressure fixability of the encapsulated toners of this invention. That is, the fixability of these encapsulated toners generally improves as the Tg of the core material decreases. It is postulated that the observed effect of a lower Tg is probably due to its effect on viscosity. A core material Tg below the fixing temperature is apparently a necessary condition for fixing since the flow or viscosity requirements for the core cannot be met above the Tg. Conversely, it seems improbable that a low Tg per se, without a concomitant reduction in viscosity, will improve the pressure fixability. As to the desirability of a high molecular weight core material, it has been postulated that a monomeric or oligomeric core material would have too low a cohesive strength to give a good fix. However, differences in fix may be attributed to the effect of core viscosity rather than to an effect of molecular weight on cohesive strength.

In addition, it has been found that there is a reasonably good correlation between the Tg of the wall material and

the toner blocking temperature. Thus, where the ratio of core material to wall material is approximately 1:1, the blocking temperature of the toner corresponds approximately to the Tg of the wall material. Crushability and pressure fixability examinations indicate that a higher molecular weight, and presumably higher strength, wall material for a given wall material such as polystyrene provides a stronger, that is, less easily crushed encapsulated toner. There is also evidence that a higher core/wall ratio provides better fixing properties, but its effect on toner crushability is indeterminate. It appears that toner crushability and fixing are affected in the same manner but in different degrees by changes in the wall and core materials as well as the core/wall ratio. In changing the wall material from low molecular weight polystyrene to the higher molecular weight polystyrenes with similar core material, or decreasing the core/wall ratio to 1:1, the fix is generally reduced but not to the extent that the crush strength is increased. Crushability measurements on encapsulated toners with relatively fluid cores agree well with the theory that crushability and impaction are directly related. Impaction of an encapsulated toner with a high molecular weight polystyrene wall is approximately one half that of a similar core material encapsulated with a low molecular weight polystyrene while the fix level is substantially equivalent.

Encapsulation of a soft adhesive in a shell material having desirable electrostatographic properties provides an electrostatographic toner which has good mechanical and electrical properties and which can be fixed on paper or other suitable transfer medium by unheated pressure rolls at low pressures. The core material is selected to provide a strong adhesive bond between the image substrate and the shell material under the conditions employed to rupture the capsules. The shell material, capsule geometry, and the shell to core ratio are selected to provide the desired electrostatographic and machine performance properties and yet permit the capsules to be ruptured at low roll pressures.

It has been found that microcapsules containing adhesive soft solids encased in a shell material such as a copolymer of styrene and a lower alkyl methacrylate or a shell material such as a polystyrene can be employed as an electrostatographic toner which can be fixed to a substrate by passage through unheated steel pressure rolls. The fixed images exhibit no tendency to smear and are nontacky under normal conditions of usage.

Any suitable encapsulation manufacturing process may be employed to produce the encapsulated toner materials of this invention. Typical encapsulation techniques are disclosed in "Microencapsulation Technology," 1969, by Dr. M. W. Ranney, Noyes Development Corporation, Park Ridge, N. J. Further, in copending patent application concurrently filed by the inventor herein, liquid, semisolid, and solid adhesive core materials may be encapsulated in a shell material by a single step atomizing and spray drying process of a single phase solution of the core and shell materials. The substantially soluble portion of a core material may be encapsulated in the substantially soluble portion of a shell material having a solubility different from the core material by dissolving the core material and the shell material in at least one relatively volatile solvent to form a solution, and substantially simultaneously forming small individual droplets of the solution, removing at least a portion of the solvent from each individual droplet by evaporation thereby increasing the concentration of the dissolved core material and the shell whereby substantially all of the core material preferentially phase separates as a solvent poor phase, and removing additional solvent from each droplet whereby the shell material deposits around the core material to form substantially dry, small spherical particles comprising the core material encapsulated with the shell material.

Basically, the above technique for the preparation of the toner materials of this invention comprises selection

of the ingredients, including the solvent or mixture of solvents, so that the change in concentration of solvent or solvents and dissolved materials during drying, and in some cases the change in pH or temperature of the atomized solution, will cause the core material to phase separate as a solvent poor, high surface tension phase in a solution of shell material. The solution of shell material will thereafter surround and encapsulate the core phase and ultimately form a substantially dry solid capsule shell upon evaporation of the solvent while the particles are 10 airborne. The separated core material phase and the separated shell material phase may be solvent poor phases and not solvent free phases. The thus produced encapsulated product can be collected in dry, free flowing form by any conventional or suitable means.

It is to be understood that although specific methods of preparing the encapsulated toner particles of this invention have been disclosed herein, other methods such as disclosed in U.S. 3,338,991 to Insalaco et al., U.S. 3,326,848 to Clemens et al., and U.S. 3,502,582 to Clemens et al. may be employed.

Any suitable adhesive, soft solid material may be employed as the core material for the encapsulated product of this invention. Typical core materials include polyesters (e.g., Epon 872, available from Shell Chemical Company), polyester based urethane polymers (e.g., Formrez P-211, P-410, P-610 available from Witco Chemical Corporation, epoxidized phenolformaldehyde resin (e.g., Epoxy-Novolak ERLB-0449, available from Union Carbide Corporation), polyisobutylene (e.g., Opipanol B-10, available from Badische Anilin & Soda Fabrik, West Germany), polyamides such as the reaction product of dimerized linoleic acid with diamines or polyamines (e.g., Versamid 100, Versamid 712, Versamid 948, and Versamid 950 available from General Mills Chemical Division and the reaction products of dimer acids with linear diamines (e.g., Emerez 1530, available from Emery Industries, Incorporated), 50/50 or 45/55 docosyl acrylate/styrene copolymers, materials which exhibit shear thinning viscosity behavior due to intermolecular hydrogen bonding such as carboxyl terminated substances prepared by the reaction of anhydrides and hydroxyl compounds, for example, the trimellitate ester of dihydroxyl terminated polycaprolactone, polyurethane elastomers (e.g., Estane 5701, 5702, 5710, and 5714 available from B. F. Goodrich Company), polyester based alkyl resins, ester gums such as rosin esters and modified rosin esters, polyvinylacetate, the polymeric reaction product of isopropylidenediphenoxypyropanol and adipic acid, the polymeric reaction product of isopropylidenediphenoxypyropanol and sebacic acid, C<sub>36</sub> di-urea and mixtures thereof.

Any suitable material may be employed as the shell material for the encapsulated product of this invention. The shell material may be a homopolymer or a copolymer of two or more monomers. Typical shell materials include: polystyrenes (e.g., PS-2, Styron 666 and Styron 678 available from Dow Chemical Company; Lustrex 99, available from Monsanto Chemical Company); poly-monochlorostyrene; copolymers such as styrene-methacrylates and styrene-acrylates; polycarbonates (e.g., Lexan 101, a poly-(4,4'-dioxydiphenyl-2,2'-propane carbonate available from General Electric Company); polyethers; low molecular weight polyethylenes; polyesters such as polymeric acrylic and methacrylic esters, fumarate polyester resins (e.g., Atlac Bisphenol A, available from Atlas Chemical Company), Dion-Iso polyester resins available from Diamond Shamrock Chemical Company, Krumbhaar polyester resins (e.g., K-2200 and K-1979, available from Lawter Chemicals, Incorporated); polyamides such as the reaction product from terephthalic acid and alkyl substituted hexamethylene diamine (e.g., Trogamid T, available from Dynamit Nobel Sales Corporation), the reaction products of dimerized linoleic acid with diamines or polyamines (e.g., Versamid 712, 75

948 and 950, available from General Mills Chemical Division), the reaction products of dimer acids, with linear diamines (e.g., Emerez 1538, 1540 and 1580 available from Emery Industries, Incorporated); naturally occurring materials such as gelatin, zein, gum arabic and the like; and mixtures thereof.

In the preparation of the encapsulated electrostatographic toner materials of this invention, although any one of many known resinous developing materials which are electroscopic in nature and which form coherent spheres when they come out of solution may be used to form the shell materials solution, it has generally been found that electrically insulating, water insoluble synthetic polymer resins form toners having many highly desirable properties, especially for use in automatic copying machines. Thus, the shell material is generally selected to provide desirable electrostatographic properties such as resistance to toner blocking, agglomeration, impact onto carrier particles, triboelectrification, crushability, and fixability. Unlike the polymeric resins used in conventional toners such as those designed for heat fusing, the shell materials for the pressure fixable toners of this invention need not necessarily be thermoplastic. In the preparation of the electrostatographic encapsulated toners of this invention, shell material resins containing a relatively high percentage of a styrene resin are preferred because they provide good image quality. The styrene resin may be a homopolymer of styrene or styrene homologues or copolymers of styrene with other monomers containing a single methylene group attached to a carbon atom by a double bond. Thus, typical monomeric materials which may be copolymerized with styrene by addition polymerization include: p-chlorostyrene; vinyl naphthalene; ethylenically unsaturated mono-olefins such as ethylene, propylene, butylene, isobutylene and the like; vinyl esters such as vinyl acetate, vinyl propionate, vinyl benzoate, vinyl butyrate and the like; esters of alpha-methylene aliphatic monocarboxylic acids such as methyl acrylate, ethyl acrylate, n-butylacrylate, isobutyl acrylate, dodecyl acrylate, n-octyl acrylate, 2-chloroethyl acrylate, phenyl acrylate, methyl-alpha-chloroacrylate, methyl methacrylate, ethyl methacrylate, propyl methacrylate, isopropyl methacrylate, butyl methacrylate and the like; acrylonitrile, methacrylonitrile; acrylamide; vinyl esters such as vinyl methyl ether, vinyl isobutyl ether, vinyl ethyl ether, and the like; vinyl ketones such as vinyl methyl ketone, vinyl hexyl ketone, methyl isopropenyl ketone and the like; vinylidene halides such as vinylidene chloride, vinylidene chlorofluoride and the like; and N-vinyl compounds such as N-vinyl pyrrole, N-vinyl carbazole, N-vinyl indole, N-vinyl pyrrolidene and the like; and mixtures thereof. The styrene resins may also be formed by the polymerization of mixtures of two or more of these unsaturated monomeric materials with a styrene monomer.

For the encapsulated electrostatographic toner materials of this invention, the shell material of the encapsulated toner should have a blocking temperature of at least about 100° F. When the encapsulated toner is characterized by a blocking temperature less than about 100° F., the toner particles may tend to agglomerate during storage and machine operation and also form undesirable films on the surface of reusable photoreceptors which adversely affect image quality. It is to be understood that the specific formulas given for units contained in the shell material resins of this invention represent the vast majority of the units present, but do not exclude the presence of monomeric units or reactants other than those which have been shown.

The ratio of shell material to core material may be any suitable value and generally is varied with the thickness, strength, porosity, and solubility characteristics of the shell desired. Thus, generally, the ratio of shell material to core material may be between about 99 parts by weight of shell material to about 1 part by weight of core material and about 1 part by weight of shell material to about

99 parts by weight of core material. However, the preferred range is between a ratio of about 7 parts by weight of shell material to about 1 part by weight of core material and about 1 part by weight of shell material to about 7 parts by weight of core material as encapsulated toner particles having the best surface characteristics are obtained. In general, the thickness of the shell material may be controlled by the ratio of the amount of core material to be encapsulated to the amount of shell material. Thus, if a thicker shell layer is desired, more shell material should be used since the ratio of shell to core material generally remains constant during the preparation of the encapsulated toner particles of this invention. In addition, the size of the encapsulated particle also generally affects the shell thickness since the smaller the particle, the smaller the shell thickness at a constant core to shell ratio.

The core, shell, or both the core and shell materials of the encapsulated toners of this invention may be pigmented or dyed, or pigmented and dyed by the addition of suitable pigment or dye or both pigment and dye to the core and shell materials. The pigment or dye, or pigment and dye, in many cases can be concentrated in the core or in the shell material or at the interface between the core and shell material. Thus, a dye may be concentrated in the phase, core or wall, in which it is soluble. The solubilities obtaining during the encapsulation could conceivably force the dye elsewhere but this would be a special case. In some cases, dyes will form separate phases like pigment particles because of insufficient solubility in the core and wall materials.

The encapsulated toners of the present invention include a colorant, either a pigment or dye, in a quantity sufficient to impart color to the resin composition, generally in a quantity up to about 25%, by weight, and particularly from about 1% to about 20%, by weight, of the toner, whereby the resulting toner will form a clearly visible image on a transfer member.

Any suitable pigment or dye or pigment and dye may be employed as the colorant for the encapsulated electrostatic toner particles of this invention. Electrostatic toner colorants are well known and include, for example, carbon black, nigrosine dye, aniline blue, Calco Oil Blue, chrome yellow, chrome green, ultramarine blue, cobalt blue, duPont Oil Red, benzidine yellow, Quinoline Yellow, methylene blue chloride, phthalocyanine blue or green, Malachite Green Oxalate, lamp black, Rose Bengal, and mixtures thereof. The pigment or dye, or pigment and dye, should be present in the toner in a sufficient quantity to render it highly colored so that it will form a clearly visible image on a recording member. Thus, for example, where conventional electrostaticographic copies of typed documents are desired, the toner may comprise a black pigment such as carbon black or a black dye such as Amaplast Black dye, available from National Aniline Products, Incorporated. Preferably, the pigment is employed in an amount from about 3 percent to about 20 percent by weight based on the total weight of the colored toner because better images are obtained. If the colorant employed is a dye, substantially smaller quantities of colorant may be used.

Obviously, the pigment need not necessarily be included in both the core and the wall of the encapsulated toner particle, but instead, may be included in only one of these or neither. Since high concentrations of pigment may adversely affect the viscous flow characteristics of some core materials, it is usually desirable that the pigment concentration below if the pigment is to be concentrated in the core. Likewise, if the pigment is to form part of the shell, the pigment concentration is preferably not so high as to inhibit the formation of an impermeable shell or otherwise adversely affect the integrity of the shell. Since the encapsulated toner particles will generally be produced in sizes ranging from about 0.5 to about 35 microns, the pigment should preferably have a diameter of less than about 0.1 micron and wherever possible should be smaller

as this contributes to the uniformity of end product coloration. In any event, the diameter of the pigment particle or other insoluble material should be about 75 percent by volume of the average core diameter.

5 Spray drying is the preferred unit operation capable of producing the encapsulated electrostaticographic toner particles of this invention. Thus, the encapsulated electrostaticographic toner particles of this invention may be prepared in the average size particle range of about 0.5 to about 1000 microns. When the encapsulated electrostaticographic toner particles of this invention are to be employed in cascade development processes, the toner should have an average particle diameter less than about 30 microns and preferably between about 5 and about 17 microns for optimum results. For use in powder cloud development methods, particle diameters of slightly less than 1 micron are preferred.

20 Suitable coated and uncoated carrier materials for cascade and magnetic brush development are well known in the art. The carrier particles may be electrically conductive, insulating, magnetic or nonmagnetic, provided that the carrier particles acquire a charge having an opposite polarity to that of the toner particles when brought in close contact with the toner particles so that the toner particles adhere to and surround the carrier particles. When a positive reproduction of an electrostatic image is desired, the carrier particle is selected so that the toner particles acquire a charge having a polarity opposite to that of the electrostatic latent image. Alternatively, if a reversal reproduction of the electrostatic image is desired, the carriers are selected so that the toner particles acquire a charge having the same polarity as that of the electrostatic image. Thus, the materials for the carrier particles are selected in accordance with their triboelectric properties in 25 respect to the electroscopic toner so that when mixed or brought into mutual contact, one component of the developer is charged positively if the other component is below the first component in the triboelectric series and negatively if the other component is above the first component in the triboelectric series. By proper selection of materials in accordance with their triboelectric effects, the polarities of their charge when mixed are such that the electroscopic toner particles adhere to and are coated on the surfaces of carrier particles and also adhere to that portion of the electrostatic image bearing surfaces having a greater attraction for the toner than do the carrier particles. Typical carriers include sodium chloride, ammonium chloride, aluminum potassium chloride, Rochelle salt, sodium nitrate, aluminum nitrate, potassium chloride, granular zircon, granular silicon, methyl methacrylate, glass, steel, nickel, iron, ferrites, ferromagnetic materials, silicon dioxide and the like. The carriers may be employed with or without a coating. Many of the foregoing and typical carriers are described by L. E. Walkup in U.S. Pat. 2,618,551; L. E. Walkup et al. in U.S. Pat. 2,638,416, E. N. Wise in U.S. Pat. 2,618,552; R. J. Hagenbach et al. in U.S. Pat. 3,591,503; and 3,533,835 and B. J. Jacknow et al. in U.S. Pat. 3,526,533. An ultimate coated carrier particle diameter between about 50 microns to about 1,000 microns is preferred because the carrier particles then possess sufficient density and inertia to avoid adherence to the electrostatic images during the cascade development process. Adherence of carrier beads to xerographic drum surfaces is undesirable because of the formation of deep scratches on the surface during the image transfer and drum cleaning steps, particularly where cleaning is accomplished by a web cleaner such as the web disclosed by W. P. Graff, Jr. et al. in U.S. Pat. 3,186,838. Also, print deletion occurs when carrier beads adhere to electrostaticographic imaging surfaces.

60 The toner compositions of the instant invention may be employed to develop electrostatic latent images on any suitable electrostatic latent image bearing surface including conventional photoconductive surfaces. Well known photoconductive materials include vitreous selenium, or-

ganic or inorganic photoconductors embedded in a non-photoconductive matrix, organic or inorganic photoconductors embedded in a photoconductive matrix, and the like. Representative patents in which photoconductive materials are disclosed include U.S. Pat. 2,803,542 to Ullrich, U.S. Pat. 2,970,906 to Bixby, U.S. Pat. 3,121,006 to Middleton, U.S. Pat. 3,121,007 to Middleton, and U.S. Pat. 3,151,982 to Corrsin.

The toner herein described is employed in a developer composition by loosely coating the toner on a suitable electrostatographic developer carrier surface to which the toner is affixed by electrostatic attraction as generally known in the art. Thus, for example, the toner composition may be employed in the cascade development technique, as more fully described in U.S. Pat. 2,618,551 to Walkup, U.S. Pat. 2,618,552 to Wise, and U.S. Pat. 2,638,416 to Walkup et al. In the cascade development technique, the developer composition is produced by mixing toner particles with a carrier which may be either electrically conducting or insulating, magnetic or nonmagnetic, provided that the carrier material when brought in close contact with the toner particles acquires a charge having an opposite polarity to that of the toner whereby the toner adheres to and surrounds the carrier. Thus, the carrier material is selected in accordance with its triboelectric properties so that the toner is either above or below the carrier material in the triboelectric series, to provide a positively or negatively charged toner.

The herein described encapsulated toners may also include other materials generally employed for modifying the characteristics of a toner, such as conductive materials to modify the triboelectric properties thereof, and the use of such materials is deemed to be within the scope of those skilled in the art from the teachings herein.

The degree of contrast or other photographic qualities in the finished image may be varied by changing the relative proportions of toner and carrier material and the choice of optimum proportions is deemed to be within the scope of those skilled in the art. In general, however, the toner of this invention is employed in amounts to provide weight ratios of carrier to toner of from about 10:1 to about 250:1, preferably from about 30:1 to about 100:1 with carrier particles of the size described above to produce a dense readily transferable image.

In addition to the use of particles to provide the carrier surface, the bristles of a fur brush may also be used. Here also, the toner particles acquire an electrostatic charge of polarity determined by the relative position of the toner particles and the fur fibers in the triboelectric series. The toner particles form a coating on the bristles of the fur clinging thereto by reason of the electrostatic attraction between the toner and the fur just as the toner clings to the surface of the carrier particles. The general process of fur brush development is described in greater detail in U.S. Pat. 3,251,706 to L. E. Walkup.

Even more closely related to the cascade carrier development is magnetic brush development. In this process, a carrier is selected having ferromagnetic properties and selective relative to the toner in a triboelectric series so as to impart the desired electrostatic polarity to the toner and carrier as in cascade carrier development. On inserting a magnet into such a mixture of toner and magnetic material, the carrier particles align themselves along the lines of force of the magnet to assume a brushlike array. The toner particles are electrostatically coated on the surface of the carrier particles. Development proceeds as in regular cascade carrier development on moving the magnet over the surface bearing the electrostatic image so that the "bristles" of the magnetic brush contact the electrostatic image bearing surface.

Still another method of carrier development is known as sheet carrier development in which the toner particles are placed on a sheet as of paper, plastic, or metal. This process is described in U.S. Pat. 2,895,847 to C. R. Mayo. As described therein, the electrostatic attraction between

the sheet surface and toner particles necessary to assure electrostatic attraction therebetween may be obtained by leading the sheet through a mass of electroscopic toner particles whereby there is obtained a rubbing or sliding contact between the sheet and the toner. In general, it is desirable to spray the surface of the sheet bearing the electroscopic toner particles with ions of the desired polarity as by the use of a corona charging device as described in the patent of Mayo. The resulting image of toner particles of the image bearing surface may then be transferred to a suitable transfer member to form the final copy. The transfer of the toner particles may be effected adhesively or electrostatically as known in the art.

The toner, as should be apparent from the hereinabove teachings, may be employed in a wide variety of developer compositions by electrostatically coating the toner composition to a suitable carrier surface, which is subsequently passed over a latent image bearing surface. The toner of the invention may also be employed for developing an electrostatic latent image formed by other than electrostatographic means; for example, the development of electrostatic latent images formed by pulsing electrodes as employed in electrostatic printing processes. In addition, the toner of the invention may be employed for developing an electrostatic latent image on a surface other than a photoconductive insulating surface. Therefore, the overall invention is not limited to a specific technique for forming or developing an electrostatic latent image or to a specific carrier for the toner.

The toners of the present invention are capable of being fixed to a suitable support medium such as paper to provide a finished copy by the application of pressure; in some cases, the pressure fixing is heat assisted, but in such cases, the amount of heat required is significantly less than that required in prior art heat fixing systems. The pressure required for effecting such pressure fixing varies with the particular toner employed. The pressure is preferably provided by pressing the transfer material having the toner image thereon between a pair of polished metal rollers that are in contact with each other under a specific pressure. It is to be understood, however, that although the toners of the present invention are particularly suitable for the preparation of a final copy by pressure fixing, such toners may also be fixed by conventional procedures; e.g., heat fusing.

A pressure fixable toner which can be fixed at low pressures to provide a fixed image comparable to those that have been fixed by heating substantially reduces fixing energy requirements, eliminates warmup time for the fixing apparatus, and also the possibility of fires caused by paper transport failures. Prior art pressure fixable toners fail to achieve these advantages because they require excessive pressures, as in the case of toners which are not encapsulated, or tend to smear because of the unfixed, broken capsules shells in the case of encapsulated liquids. The use of an adhesive core coupled with provision for adjustment of the electrostatographic properties of the shell permits attaining the desired fixing properties of the toner material without smearing of the ruptured shells by bonding the shells tightly to the paper. The diffusion of a liquid core material through the capsule shell, even though too slight to cause a serious loss of core material in storage, can cause variable electrostatographic properties. Another advantage of the encapsulated soft-solids of this invention over encapsulated liquids is that the molecular size and physical properties of these soft-solids prevent diffusion of the core material through the shell.

## 70 DESCRIPTION OF PREFERRED EMBODIMENTS

This invention is further illustrated by the following examples but it is to be understood that the scope of the invention is not to be limited thereby. Unless otherwise specified, all parts are by weight.

In the following examples, the term "stick point" means the temperature at which a material adheres to a metallic substrate; for example, a continuous line of sample is equilibrated on a Kofler Hot Bench for about 2 hours and then gently brushed away. The "stick point" is the lowest temperature at which the sample "sticks" to the metallic plate of the hot bench. Likewise, the term "blocking tests" refers to tests usually conducted on small open dishes of toner material at specific temperature conditions. The blocking temperature is determined as the lowest temperature to which the toner has been subjected for a period of equilibration and the "crusty" mass produced can no longer be easily broken down to the original particles. Also, the term "geometric standard deviation" is the deviation encountered in a particle size analysis, approximately measured as the ratio of the particle diameter which is greater than that of 84% of the sample to the particle diameter which is greater than that of 50% of the sample. In addition, the term "Taber Cycles" is the degree of fix obtained using a test method based on the resistance of a fixed toner image to abrasion with a Taber Abrader. A standard test pattern is printed at conditions to provide an integrated optical density as determined by a Welch Densitometer (Model 3834) of  $1.2 \pm 0.1$ . The test pattern is pressure fixed and then abraded with a weight of 375 grams on the abrader arm until the measured density is 80 percent of the initial density. The result is given as the number of "Taber Cycles" required to reduce the initial density by 20 percent.

## Example I

30

A control toner mixture is prepared comprising about 5 parts by weight of carbon black and about 95 parts by weight of a polymeric condensation product of 2,2 bis(4-hydroxy-isopropoxy-phenyl)-propane and fumaric acid. This polymer has a number average molecular weight of about 8000. After melting and preliminary mixing, the composition is fed into a rubber mill and thoroughly milled to yield a uniformly dispersed composition of the carbon black in the thermoplastic resin body. The resulting mixed composition is cooled and then finely subdivided in a jet pulverizer to yield toner particles having an average particle size of about 7 to about 12 microns. About 1 part by weight of the pulverized toner particles are mixed with about 99 parts by weight of 250 micron glass carrier beads. Prints were made to provide an integrated optical density of  $1.2 \pm 0.1$  in a modified Xerox 660 Copier having the fuser removed. Pressure fixing was performed in an apparatus having two steel rolls of about 3 inches each in diameter in contact with each other. The contact pressure between the two rolls may be varied as desired up to approximately 500 p.l.i. The upper steel roll may be heated externally with a 2000 watt quartz infrared lamp. The fuser temperature is regulated with a proportional temperature controller and is monitored by means of a thermistor in sliding contact with the center of the upper fuser roll. The prints made were then pressure fixed at 300 and 400 p.l.i. respectively with the assistance of heat at temperatures between about 110° F. and 140° F. in 10° F. increments. After passage through the fuser, the prints were evaluated for degree of fix in terms of Taber Cycles. The results of these tests are summarized in the following table:

| FIX (TABER CYCLES) |     |     |
|--------------------|-----|-----|
| Pressure, p.l.i.   | 300 | 400 |
| Temperature, ° F.: |     |     |
| 110                | 1.0 | 2.0 |
| 120                | 1.0 | 2.0 |
| 130                | 1.5 | 2.0 |
| 140                | 2.0 | 3.5 |

## Example II

An encapsulated toner material is prepared from a solution comprising about 300 grams of a polystyrene (PS-2) and about 300 grams of polyhexamethylene seba-

cate having a weight average molecular weight of about 24,000 in a mixture of cyclohexane and chloroform at a 4.0:1.0 cyclohexane:chloroform volume ratio. A carbon black is dispersed in the solution by severe agitation. The final concentrations are about 2.4 percent polystyrene, about 2.4 percent polyhexamethylene sebacate, about 0.2 percent carbon black, and about 95.0 percent solvent. The solution, with dispersed carbon black, is spray dried using a Bowen Engineering, Incorporated, five foot diameter spray dryer with a spinning disk atomizer operating at about 30,000 r.p.m. and a feed rate of about 200 ml./minute. Drying air inlet temperature is about 130° F. and outlet air temperature is about 101° F. The dry product is a powder of about 15.9 micron diameter volume average particle size with a geometric standard deviation of about 2.17. Electron and/or optical microscope examination shows the individual particles to be primarily spherical and to have a pigmented core surrounded by a substantially clear shell. Stick point, blocking tests, and examination of crushed particles with the scanning electron microscope all indicate that the shell is principally polystyrene and the core principally polyhexamethylene sebacate and carbon black. About 1 part by weight of the encapsulated toner particles were mixed with about 99 parts by weight of 250 micron glass carrier beads and substituted for the developer in the testing machine described in Example I. Under substantially identical test conditions, the following degree of fix in terms of Taber Cycles is obtained.

## FIX (TABER CYCLES)

| Pressure, p.l.i.   | 300 | 400 |
|--------------------|-----|-----|
| Temperature, ° F.: |     |     |
| 110                | 4.2 | 5.0 |
| 120                | 5.5 | 6.0 |

From the above results, it is seen that this encapsulated toner composition exhibits a greater degree of fix than the control toner mixture of Example I at substantially the same fixing pressures and temperatures.

## Example III

An encapsulated toner material is prepared from a solution comprising about 900 grams of a polystyrene (Styron 678) and about 900 grams of the reaction product of isopropylidenediphenoxypopropanol and sebacic acid having a number average molecular weight of about 2230 in a mixture of heptane and chloroform at a 1.3:1.0 heptane:chloroform volume ratio and a 1:1 core to wall ratio. A carbon black is dispersed in the solution by severe agitation. The final concentrations are about 2.4 percent polystyrene, about 2.4 percent reaction product of isopropylidenediphenoxypopropanol and sebacic acid, about 0.2 percent carbon black, and about 95.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 160° F. and outlet air temperature is about 125° F. The dry product is a powder of about 16.7 micron diameter volume average particles size with a geometric standard deviation of about 1.67. Electron and/or optical microscope examination shows the individual particles to be primarily spherical and to have a pigmented core surrounded by a substantially clear shell. Stick point blocking tests, and examination of crushed particles with the scanning electron microscope all indicate that the shell is principally polystyrene and the core principally the reaction product of isopropylidenediphenoxypopropanol and sebacic acid and carbon black. About 1 part by weight of the encapsulated toner particles were mixed with about 99 parts by weight of 250 micron glass carrier beads and substituted for the developer in the testing machine described in Example I. Under substantially identical test

conditions, the following degree of fix in terms of Taber Cycles is obtained.

| FIX (TABER CYCLES) |     |      |
|--------------------|-----|------|
| Pressure, p.l.i.   | 300 | 400  |
| Temperature, ° F.: |     |      |
| 110.....           | 4.5 | 6.0  |
| 120.....           | 4.5 | 10.0 |

From the above results, it is seen that this encapsulated toner composition exhibits a degree of fix greater than the control toner mixture of Example I at substantially the same fixing pressures and temperatures. In addition, it was determined that this toner composition fixed at 75° F. provided about the same degree of fix as the control composition of Example I which was fixed at 120° F. and corresponding pressure.

#### Example IV

An encapsulated toner material is prepared from a solution comprising about 647 grams of a polystyrene (PS-2) and about 647 grams of a polyethylene azelate having a melting point of between about 40° C. and about 50° C. in a mixture of cyclohexane and chloroform at a 2.0:1.0 cyclohexane-chloroform volume ratio. A carbon black is dispersed in the solution by severe agitation. The final concentrations are about 2.4 percent polystyrene, about 2.4 percent polyethylene azelate, about 0.2 percent carbon black, and about 95.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 135° F. and outlet air temperature is about 110° F. The dry product is a powder of about 17.8 micron diameter volume average particle size with a geometric standard deviation of about 1.74. Electron and/or optical microscope examination shows the individual particles to be primarily spherical and to have a pigmented core surrounded by a substantially clear shell. Stick point, blocking tests and examination of crushed particles with the scanning electron microscope all indicate that the shell is principally polystyrene and the core principally polyethylene azelate and carbon black. About 1 part by weight of the encapsulated toner particles were mixed with about 99 parts by weight of 250 micron glass carrier beads and substituted for the developer in the testing machine described in Example I. Under substantially identical test conditions, the following degree of fix in terms of Taber Cycles is obtained.

| FIX (TABER CYCLES) |      |      |
|--------------------|------|------|
| Pressure, p.l.i.   | 300  | 400  |
| Temperature, ° F.: |      |      |
| 110.....           | 36.6 | 34.0 |
| 120.....           | 37.3 | 38.6 |

From the above results, it is seen that this encapsulated toner composition exhibits a much greater degree of fix than the control toner mixture of Example I at substantially the same fixing pressures and temperatures.

#### Example V

An encapsulated toner material is prepared from a solution comprising about 9.5 pounds of a polystyrene (PS-2) and about 9.5 pounds of the reaction product of isopropylidenediphenoxypopropanol and adipic acid having a number average molecular weight of about 3100 in a mixture of chloroform and heptane at a 1:1.3 chloroform:heptane volume ratio. A carbon black is dispersed in the solution by severe agitation. The final concentrations are about 4.75 percent polystyrene, about 4.75 percent reaction product of isopropylidenediphenoxypopro-

panol and adipic acid, about 0.5 percent carbon black, and about 90.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 210° F. and outlet air temperature is about 160° F. The dry product is a powder of about 12.7 micron diameter volume average particle size with a geometric standard deviation of about 1.58. Electron and/or optical microscope examination shows the individual particles to be primarily spherical and to have a pigmented core surrounded by a substantially clear shell. Stick point, blocking tests, and examination of crushed particles with the scanning electron microscope all indicate that the shell is principally polystyrene and the core principally the reaction product of isopropylidenediphenoxypopropanol and adipic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints were pressure fixed without the assistance of heat, the degree of fix is found to be about 2.0 Taber Cycles at 300 p.l.i. of pressure and about 3.8 at 400 p.l.i. of pressure. Thus, it is seen that this toner composition provides a degree of fix equivalent to that of the toner composition of Example I at comparable pressures and at ambient temperature compared with that obtained at a temperature of 140° F. employed in fixing the toner composition of Example I.

#### Example VI

An encapsulated toner material is prepared from a solution comprising about 300 grams of a polystyrene (PS-2) and about 300 grams of epoxidized phenolformaldehyde resin (Epoxy-Novolak ERLB-0449) having a number average molecular weight of about 700 in a mixture of chloroform and cyclohexane at a 1:0.75 chloroform: cyclohexane volume ratio. A carbon black is dispersed in the solution by severe agitation. The final concentrations are about 4.75 percent polystyrene, about 4.75 percent epoxidized phenolformaldehyde, about 0.5 percent carbon black, and about 90.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 155° F. and outlet air temperature is about 127° F. The dry product is a powder of about 13.0 micron diameter volume average particle size with a geometric standard deviation of about 1.61. Electron and/or optical microscope examination shows the individual particles to be primarily spherical and to have multiple pigmented cores surrounded by and embedded in a substantially clear shell material. Stick point, blocking tests and examination of crushed particles with the scanning electron microscope all indicate that the shell is principally polystyrene and the cores principally epoxidized phenolformaldehyde and carbon black. About 1 part by weight of the encapsulated toner particles were mixed with about 99 parts by weight of 250 micron glass carrier beads and substituted for the developer in the testing machine described in Example I. Under substantially identical test conditions, except that the prints were pressure fixed without the assistance of heat, the degree of fix is found to be about 3.1 Taber Cycles at 300 p.l.i. of pressure and about 5.8 Taber cycles at 500 p.l.i. of pressure. Thus, it is seen that this toner composition provides a degree of fix greater than that of the toner composition of Example I at both 300 and 500 p.l.i. of pressure and at ambient temperature compared with that obtained at a temperature of 140° F. employed in fixing the toner composition of Example I.

An encapsulated toner material is prepared from a solution comprising about 400 grams of a fractionated polystyrene and about 400 grams of the reaction product of isopropylidenediphenoxypopropanol and adipic acid having a number average molecular weight of about 2100 in a mixture of chloroform and heptane at a 1:1.3 chloroform:heptane volume ratio. A carbon black is dispersed in the solution by severe agitation. The final concentrations are about 4.75 percent polystyrene, about 4.75 percent reaction product of isopropylidenediphenoxypopropanol and adipic acid, about 0.5 percent carbon black, and about 90.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 200° F. and outlet air temperature is about 170° F. The dry product is a powder of about 12.6 micron diameter volume average particle size with a geometric standard deviation of about 1.87. Electron and/or optical microscope examination shows the individual particles to be primarily spherical and to have a pigmented core surrounded by a substantially clear shell. Stick point, blocking tests and examination of crushed particles with the scanning electron microscope all indicate that the shell is principally polystyrene and the core principally the reaction product of isopropylidenediphenoxypopropanol and adipic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints were fixed without the assistance of heat, the degree of fix obtained was found to be about 1.5 Taber Cycles at 300 p.l.i. of pressure and about 3.2 Taber Cycles at 500 p.l.i. of pressure. Thus, it is seen that this toner composition provides a degree of fix almost equivalent to that of the toner composition of Example I at 300 and 500 p.l.i. of pressures and at ambient temperature compared with that obtained at a temperature of 140° F. employed in fixing the toner composition of Example I.

## Example VIII

An encapsulated toner material is prepared from a solution comprising about 363 grams of a polystyrene (PS-2) and about 437 grams of epoxidized phenolformaldehyde (Epoxy-Novolak ERLB-0449) having a number average molecular weight of about 700 in a mixture of chloroform and cyclohexane at a 4:3 chloroform:cyclohexane volume ratio. A carbon black is dispersed in the solution by severe agitation. The final concentrations are about 4.3 percent polystyrene, about 5.2 percent epoxidized phenolformaldehyde, about 0.5 percent carbon black, and about 90.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 145° F. and outlet air temperature is about 125° F. The dry product is a powder of about 15.0 micron diameter volume average size with a geometric standard deviation of about 1.53. Electron and/or optical microscope examination shows the individual particles to be primarily spherical and to have pigmented cores surrounded by and embedded in a substantially clear shell material. Stick point, blocking tests, and examination of crushed particles with the scanning electron microscope all indicate that the shell is principally polystyrene and the cores principally epoxidized phenolformaldehyde and carbon black. About 1 part by weight of the encapsulated toner particles were mixed with about 99 parts by weight of 250 micron glass carrier beads and substi-

tuted for the developer in the testing machine described in Example I. Under substantially identical test conditions, except that the prints made were pressure fixed without the assistance of heat, the degree of fix obtained was found to be about 3.2 Taber Cycles at 300 p.l.i. of pressure and about 6.2 Taber Cycles at 500 p.l.i. of pressure. From these results, it is seen that this toner composition provides a degree of fix substantially greater than that of the toner composition of Example I at 300 and 500 p.l.i. pressures and at ambient temperature compared with that obtained at a temperature of 140° F. employed in fixing the toner composition of Example I.

## Example IX

An encapsulated toner material is prepared from a solution comprising about 400 grams of polystyrene (PS-2) and about 400 grams of the reaction product of isopropylidenediphenoxypopropanol and sebacic acid having a number average molecular weight of about 2230 in a mixture of chloroform and cyclohexane at a 1:3 chloroform:cyclohexane volume ratio. A carbon black is dispersed in the solution by severe agitation. The final concentrations are about 4.75 percent polystyrene, about 4.75 percent reaction product of isopropylidenediphenoxypopropanol and sebacic acid, about 0.5 percent carbon black, and about 90.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 145° F. and outlet air temperature is about 120° F. The dry product is a powder of about 13.3 micron diameter volume average particle size with a geometric standard deviation of about 1.75. Electron and/or optical microscope examination shows the individual particles to be primarily spherical and to have a pigmented core surrounded by a substantially clear shell. Stick point, blocking tests and examination of crushed particles with the scanning electron microscope all indicate that the shell is principally polystyrene and the core principally the reaction product of isopropylidenediphenoxypopropanol and sebacic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained was found to be about 27 Taber Cycles at 300 p.l.i. of pressure and about 86 Taber Cycles at 500 p.l.i. pressure. From these results, it is seen that this toner composition provides a degree of fix which is significantly greater than that of the toner composition of Example I at 300 and 500 p.l.i. pressures and at ambient temperature compared with that obtained at a temperature of 140° F. employed in fixing the toner composition of Example I.

## Example X

An encapsulated toner material is prepared from a solution comprising about 300 grams of a polystyrene (Styron 678) and about 300 grams of the reaction product of isopropylidenediphenoxypopropanol and adipic acid having a number average molecular weight of about 1780 in a mixture of chloroform and heptane at a 1:1.3 chloroform:heptane volume ratio. A carbon black is dispersed in the solution by severe agitation. The final concentrations are about 2.4 percent polystyrene, about 2.4 percent reaction product of isopropylidenediphenoxypopropanol and adipic acid, about 0.2 percent carbon black, and about 95.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is between about 160° F. and 143° F. and outlet

air temperature is between about 125° F. and about 115° F. The dry product is a powder of about 15.1 micron diameter volume average particle size with a geometric standard deviation of about 1.66. Electron and/or optical microscope examination shows the individual particles to be primarily spherical and to have a pigmented core surrounded by a substantially clear shell. Stick point, blocking tests, and examination of crushed particles with the scanning electron microscope all indicate that the shell is principally polystyrene and the core principally the reaction product of isopropylidenediphenoxypopropanol and adipic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained was found to be about 1.5 Taber Cycles at 300 p.l.i. of pressure and about 3.4 Taber Cycles at 500 p.l.i. of pressure. Thus, it is seen that this toner composition provides a degree of fix substantially equivalent to that of the toner composition of Example I at 300 and 500 p.l.i. of pressure and at ambient temperature compared with that obtained at a temperature of 140° F. employed in fixing the toner composition of Example I.

#### Example XI

An encapsulated toner material is prepared from a solution comprising about 250 grams of a polystyrene (Styron 678) and about 500 grams of the reaction product of isopropylidenediphenoxypopropanol and adipic acid having a number average molecular weight of about 1780 in a mixture of chloroform and heptane at a 1:1.3 chloroform:heptane volume ratio. A carbon black is dispersed in the solution by severe agitation. The final concentrations are about 1.6 percent polystyrene, about 3.2 percent reaction product of isopropylidenediphenoxypopropanol and adipic acid, 0.2 percent carbon black, and about 95.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 142° F. and outlet air temperature is about 113° F. The dry product is a powder of about 12.3 micron diameter volume average particle size with a geometric standard deviation of about 1.58. Electron and/or optical microscope examination shows the individual particles to be primarily spherical and to have a pigmented core surrounded by a substantially clear shell. Stick point, blocking test, and examination of crushed particles with the scanning electron microscope all indicate that the shell is principally polystyrene and the core principally the reaction product of isopropylidenediphenoxypopropanol and adipic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained was found to be about 4.4 Taber Cycles at 300 p.l.i. of pressure and about 9.7 Taber Cycles at 500 p.l.i. of pressure. From these results, it is seen that this toner composition provides a degree of fix more than twice as great as that of the toner composition of Example I at 300 and 500 p.l.i. pressures and at ambient temperature compared with that obtained at a temperature of 140° F. employed in fixing the toner composition of Example I.

#### Example XII

An encapsulated toner material is prepared from a solution comprising about 200 grams of the reaction product of a dimer acid with a linear diamine (Emerez 1540, Emery Industries, Incorporated) and about 200

grams of the reaction product of isopropylidenediphenoxypopropanol and adipic acid having a number average molecular weight of about 1780 in a mixture of chloroform and isopropanol at a 1:2 chloroform: isopropanol volume ratio. A carbon black is dispersed in the solution by severe agitation. The final concentrations are about 4.8% reaction product of the dimer acid with a linear diamine, about 4.8% reaction product of isopropylidene-diphenoxypopropanol and adipic acid, about 0.5% carbon black, and about 90.0% solvent. The solution, with dispersed carbon black, is spray dried using a Bowen Engineering, Incorporated, laboratory model 30 inch diameter spray dryer with a spinning disk atomizer operating at about 50,000 r.p.m. and a feed rate of about 200 ml./minute. Drying air inlet temperature is about 151° F. and outlet air temperature is about 118° F. The dry product is a powder of about 11.6 micron diameter volume average particle size with a geometric standard deviation of about 1.56. Electron and/or optical microscope examination shows the individual particles to be primarily spherical and to have a pigmented core surrounded by a clear shell. Stick point, blocking tests and examination of crushed particles with the scanning electron microscope all indicate that the shell is principally the reaction product of a dimer acid with a linear diamine and the core principally the reaction product of isopropylidenediphenoxypopropanol and adipic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained was found to be about 1.4 Taber Cycles at 300 p.l.i. of pressure and about 3.3 Taber Cycles at 500 p.l.i. of pressure. From these results, it is seen that this toner composition provides a degree of fix slightly less than that of the toner composition of Example I at 300 and 500 p.l.i. of pressure and at ambient temperature compared with that obtained at a temperature of 140° F. employed in fixing the toner composition of Example I. In addition, this toner printed reversal and gave good, high density prints using a reversal image. An excellent encapsulation was achieved with these toner materials.

#### Example XIII

An encapsulated toner material is prepared from a solution comprising about 375 grams of a polystyrene (PS-2) and about 375 grams of the reaction product of isopropylidenediphenoxypopropanol and sebacic acid having a number average molecular weight of about 4110 in a mixture of chloroform and cyclohexane at a 1:3 chloroform:cyclohexane volume ratio. A carbon black is dispersed in the solution by severe agitation. The final concentrations are about 4.75 percent polystyrene, about 4.75 percent reaction product of isopropylidenediphenoxypopropanol and sebacic acid, about 0.5 percent carbon black, and about 90.0 percent solvent. The solution, with dispersed carbon black, is spray dried using a Bowen Engineering, Incorporated, laboratory model 30 inch diameter spray dryer with a spinning disk atomizer operating at about 50,000 r.p.m. and a feed rate of about 200 ml./minute. Drying air inlet temperature is about 145° F. and outlet air temperature is about 120° F. The dry product is a powder of about 15:1 micron diameter volume average particle size with a geometric standard deviation of about 1.86. Electron and/or optical microscope examination shows the individual particles to be primarily spherical and to have a pigmented core surrounded by a substantially clear shell. Stick point, blocking tests and examination of crushed particles with the scanning electron microscope all indicate that the shell is principally polystyrene and the core principally the reaction product of isopropylidenediphenoxypopropanol and sebacic acid and carbon black. About 1 part by weight of the encapsulated

toner particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained was found to be about 3.0 Taber Cycles at 200 p.l.i. of pressure and about 13.5 Taber Cycles at 500 p.l.i. of pressure. From these results, it is seen that this toner composition provides a degree of fix significantly greater than that obtained with the toner composition of Example I at 200 and 500 p.l.i. pressures and at ambient temperature compared with that obtained at a temperature of about 140° F. employed in fixing the toner composition of Example I.

#### Example XIV

An encapsulated toner material is prepared from a solution comprising about 320 grams of a polystyrene (PS-2) and about 320 grams of the reaction product of isopropylidenediphenoxypopropanol and sebacic acid having a number average molecular weight of about 2410 in a mixture of chloroform and cyclohexane at a 1:3 chloroform:cyclohexane volume ratio. Neospectra Mark II, a carbon black, is dispersed in the solution by severe agitation. The final concentrations are about 4.75 percent polystyrene, about 4.75 percent reaction product of isopropylidenediphenoxypopropanol and sebacic acid, about 0.5 percent carbon black, and about 90.0 percent solvent. The solution, with dispersed carbon black, is spray dried using a Bowen Engineering, Incorporated, laboratory model 30 inch diameter spray dryer with a spinning disk atomizer operating at about 50,000 r.p.m. and a feed rate of about 200 ml./minute. Drying air inlet temperature is about 146° F. and outlet air temperature is about 118° F. The dry product is a powder of about 16.8 micron diameter volume average particle size with a geometric standard deviation of about 1.67. Electron and/or optical microscope examination shows the individual particles to be primarily spherical and to have a pigmented core surrounded by a substantially clear shell. Stick point, blocking tests and examination of crushed particles with the scanning electron microscope all indicate that the shell is principally polystyrene and the core principally the reaction product of isopropylidenediphenoxypopropanol and sebacic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained was found to be about 10.5 Taber Cycles at 300 p.l.i. of pressure and about 22.0 Taber Cycles at 500 p.l.i. of pressure. From these results, it is seen that this toner composition provides a degree of fix significantly greater than that obtained with the toner composition of Example I at 300 and 500 p.l.i. pressures and at ambient temperature compared with a temperature of 140° F. employed in fixing the toner composition of Example I.

#### Example XV

An encapsulated toner material is prepared from a solution comprising about 800 grams of a polystyrene (PS-2) and about 800 grams of the reaction product of isopropylidenediphenoxypopropanol and sebacic acid having a number average molecular weight of about 2230 in a mixture of chloroform and cyclohexane at a 1:3 chloroform:cyclohexane volume ratio. A carbon black is dispersed in the solution by severe agitation. The final concentrations are about 4.75 percent polystyrene, about 4.75 percent reaction product of isopropylidenediphenoxypopropanol and sebacic acid, about 0.5 percent carbon black, and about 90.0 percent solvent. The solution, with dispersed carbon black, is spray dried using a Bowen Engi-

neering, Incorporated, five foot diameter spray dryer with a spinning disk atomizer operating at about 50,000 r.p.m. and a feed rate of about 200 ml./minute. Drying air inlet temperature is about 148° F. and outlet air temperature is about 118° F. The dry product is a powder of about 17.0 micron diameter volume average particle size with a geometric standard deviation of about 1.73. Electron and/or optical microscope examination shows the individual particles to be primarily spherical and to have a pigmented core surrounded by a substantially clear shell. Stick point, blocking tests and examination of crushed particles with the scanning electron microscope all indicate that the shell is principally polystyrene and the core principally the reaction product of isopropylidenediphenoxypopropanol and sebacic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained is found to be about 33.0 Taber Cycles at 400 p.l.i. of pressure and about 43.0 Taber Cycles at 500 p.l.i. of pressure. From these results, it is seen that this toner composition provides a degree of fix significantly greater than that of the toner composition of Example I at 400 and 500 p.l.i. pressures and at ambient temperature compared with that obtained at a temperature of 140° F. employed in fixing the toner composition of Example I.

#### Example XVI

An encapsulated toner material is prepared from a solution comprising about 119 grams of a polystyrene (Styron 678) and about 119 grams of the reaction product of isopropylidenediphenoxypopropanol and sebacic acid having a number average molecular weight of about 2230 in a mixture of ethylene dichloride and cyclohexane at a 1:2.2 ethylene dichloride:cyclohexane volume ratio. A carbon black is dispersed in the solution by severe agitation. The final concentrations are about 1.4 percent polystyrene, about 1.4 percent reaction product of isopropylidenediphenoxypopropanol and sebacic acid, about 0.2 percent carbon black, and about 97.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 138° F. and outlet air temperature is about 110° F. The dry product is a powder of about 11.0 micron diameter volume average particle size with a geometric standard deviation of about 1.82. Electron and/or optical microscope examination shows the individual particles to be primarily spherical and to have a pigmented core surrounded by a substantially clear shell. Stick point, blocking tests, and examination of crushed particles with the scanning electron microscope all indicate that the shell is principally polystyrene and the core principally the reaction product of isopropylidenediphenoxypopropanol and sebacic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained is found to be about 6.25 Taber Cycles at 400 p.l.i. of pressure and about 8.75 Taber Cycles at 500 p.l.i. of pressure. From these results, it is seen that this toner composition provides a degree of fix approximately three times that of the toner composition of Example I at 400 and 500 p.l.i. pressures and at ambient temperature compared with that obtained at a temperature of 140° F. employed in fixing the toner composition of Example I.

## Example XVII

An encapsulated toner material is prepared from a solution comprising about 95 grams of a polystyrene (Styron 678) and about 142 grams of the reaction product of isopropylidenediphenoxypopropanol and sebacic acid having a number average molecular weight of about 2230 in a mixture of ethylene dichloride and cyclohexane at a 1:2.2 ethylene dichloride:cyclohexane volume ratio. A carbon black is dispersed in the solution by severe agitation. The final concentrations are about 1.2 percent polystyrene, about 1.8 percent reaction product of isopropylidenediphenoxypopropanol and sebacic acid, about 0.2 percent carbon black, and about 96.8 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 136° F. and outlet air temperature is about 107° F. The dry product is a powder of about 7.9 micron diameter volume average particle size with a geometric standard deviation of about 1.75. Electron and/or optical microscope examination shows the individual particles to be primarily spherical and to have a pigmented core surrounded by a substantially clear shell. Stick point, blocking tests and examination of crushed particles with the scanning electron microscope all indicate that the shell is principally polystyrene and the core principally the reaction product of isopropylidenediphenoxypopropanol and sebacic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained was about 6.0 Taber Cycles at 400 p.l.i. of pressure and about 8.3 Taber Cycles at 500 p.l.i. of pressure. From these results, it is seen that this toner composition provides a degree of fix almost three times greater than that of the toner composition of Example I at 400 and 500 p.l.i. pressures and at ambient temperature compared with that obtained at a temperature of 140° F. employed in fixing the toner composition of Example I.

## Example XVIII

An encapsulated toner material is prepared from a solution comprising about 1600 grams of a polystyrene (PS-2) and about 1600 grams of the reaction product of isopropylidenediphenoxypopropanol and sebacic acid having a number average molecular weight of about 2230 in a mixture of chloroform and cyclohexane at a 1:3 chloroform:cyclohexane volume ratio. A carbon black is dispersed in the solution by severe agitation. The final concentrations are about 4.75 percent polystyrene, about 4.75 percent reaction product of isopropylidenediphenoxypopropanol and sebacic acid, about 0.5 percent carbon black, and about 90.0 percent solvent. The solution, with dispersed carbon black, is spray dried using a Bowen Engineering, Incorporated, five foot diameter spray dryer with a spinning disk atomizer operating at about 50,000 r.p.m. and a feed rate of about 200 ml./minute. Drying air inlet temperature is about 143° F. and outlet air temperature is about 115° F. The dry product is a powder of about 18.5 micron diameter volume average particle size with a geometric standard deviation of about 1.62. Electron and/or optical microscope examination shows the individual particles to be primarily spherical and to have a pigmented core surrounded by a substantially clear shell. Stick point, blocking tests, and examination of crushed particles with the scanning electron microscope all indicate that the shell is principally polystyrene and the core principally the reaction product of isopropylidenediphenoxypopropanol and sebacic acid and carbon black. About 1 part by weight of the encapsulated toner

particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained is found to be about 58.5 Taber Cycles at 400 p.l.i. of pressure and about 67.0 Taber Cycles at 500 p.l.i. of pressure. From these results, it is seen that this toner composition provides a degree of fix substantially greater than that of the toner composition of Example I at 400 and 500 p.l.i. pressures and at ambient temperature compared with that obtained at a temperature of 140° F. employed in fixing the toner composition of Example I.

## Example XIX

An encapsulated toner material is prepared from a solution comprising about 190 grams of a polystyrene (Styron 678) and about 284 grams of the reaction product of isopropylidenediphenoxypopropanol and sebacic acid having a number average molecular weight of about 2230 in a mixture of ethylene dichloride and cyclohexane at a 2.2:1 ethylene dichloride:cyclohexane volume ratio. A carbon black is dispersed in the solution by severe agitation. The final concentrations are about 1.1 percent polystyrene, about 1.7 percent reaction product of isopropylidenediphenoxypopropanol and sebacic acid, about 0.2 percent carbon black, and about 97.0 percent solvent. The solution, with dispersed carbon black is spray dried using a Bowen Engineering, Incorporated, five foot diameter spray dryer with a spinning disk atomizer operating at about 50,000 r.p.m. and a feed rate of about 200 ml./minute. Drying air inlet temperature is about 137° F. and outlet air temperature is about 110° F. The dry product is a powder of about 10.4 micron diameter volume average particle size with a geometric standard deviation of about 1.81. Electron and/or optical microscope examination shows the individual particles to be primarily spherical and to have a pigmented core surrounded by a substantially clear shell. Stick point, blocking tests, and examination of crushed particles with the scanning electron microscope all indicate that the shell is principally polystyrene and the core principally the reaction product of isopropylidenediphenoxypopropanol and sebacic acid and carbon black. About 1 part by weight of the encapsulated toner particles were mixed with about 99 parts by weight of 250 micron glass carrier beads and substituted for the developer in the testing machine described in Example I. Under substantially identical test conditions, except that the prints made were pressure fixed without the assistance of heat, the degree of fix obtained is about 7.0 Taber Cycles at 400 p.l.i. of pressure and about 8.8 Taber Cycles at 500 p.l.i. of pressure. From these results, it is seen that this toner composition provides a degree of fix approximately three times that of the toner composition of Example I at 400 and 500 p.l.i. pressures and at ambient temperature compared with that obtained at a temperature of 140° F. employed in fixing the toner composition of Example I.

## Example XX

A test was conducted to determine whether copies made with the encapsulated toner material of Example V pressure fixed at different p.l.i. levels and image densities would offset to another copy or to a blank sheet of paper. Copies at image density levels of 0.7, 1.2 and 1.4 were fixed at about 100 through about 500 p.l.i. of pressure and placed under a load of about 3.42 pounds and stored in an office building where the temperature varied between about 60° F. and about 85° F. The copies were checked periodically over an eight month period without any observation of copy to copy offset. The following table summarizes the fix levels obtained in Taber Cycles at pressures

between about 100 and about 500 p.l.i. one hour after fix and also for eight months after fix.

| TABER CYCLES       |                    |                       |
|--------------------|--------------------|-----------------------|
|                    | 1 hr. after<br>fix | 8 months<br>after fix |
| Pressure (p.l.i.): |                    |                       |
| 100 -----          | 1.0                | 9                     |
| 200 -----          | 1.3                | 10                    |
| 300 -----          | 2.0                | 35                    |
| 400 -----          | 2.5                | 43                    |
| 500 -----          | 3.0                | 45                    |

### Example XXI

An experiment was conducted to determine whether the flow properties of the toner material of Example V could be improved. Poor toner flowability can become a major problem in toner packaging and toner dispensing. Thus, the flowability of the toner material of Example V with various amounts of a powdered hydrophobic silica, Aerosil R-972, was studied relative to Xerox 364 toner. Flowability was measured by determining the amount of toner which would pass through a sieve under controlled conditions. The results obtained agree with the observed dispensing behavior in simulated machine testing. Thus, the silica was dispersed in the toner at concentrations from about 0.02% to about 1.0% by weight of the toner by tumbling the samples end over end in a can tumbler. The triboelectric values for the samples were measured versus homogeneous 450 micron glass carrier beads. The developers were roll-milled in 8 ounce glass jars for three hours, and triboelectric measurements were made at 10, 30 and 180 minutes. The data obtained indicated that much less than 1% silica is sufficient to greatly increase the toner flowability and markedly effect the triboelectric characteristics of the toner. It was found that the addition of about 0.02% of silica provides a toner flowability comparable to Xerox 364 toner. The addition of 0.1% silica substantially improved the stability of the triboelectric properties of the toner material of Example V with time and also provided an acceptable triboelectric value. There was also evidence that the addition of silica reduces triboelectric variations between different batches of the toner material of Example V. The addition of the powdered silica noticeably improved the flowability of the toner material of Example V in machine testing. The addition of silica also produced a high, stable triboelectricity.

### Example XXII

An encapsulated toner material is prepared from a solution comprising about 431 grams of a polystyrene (Styron 678) and about 431 grams of the reaction product of isopropylidene-diphenoxypyropanol and adipic acid having a number average molecular weight of about 3275 in a mixture of chloroform and heptane at a 1:1.3 chloroform:heptane volume ratio. A tetra-isohexyl-sulfonamido copper phthalocyanine dye is dissolved in the solution by agitation. The final concentrations are about 4.8% polystyrene, about 4.9% reaction product of isopropylidene-diphenoxypyropanol and adipic acid, about 0.5% phthalocyanine dye, and about 90.0% solvent. The solution is spray dried using a Bowen Engineering, Incorporated, laboratory model 30 inch diameter spray dryer with a spinning disk atomizer operating at about 50,000 r.p.m. and a feed rate of about 200 ml./minute. Drying air inlet temperature is about 157° F. and outlet air temperature is about 134° F. The dry product is a powder of about 14.8 micron diameter volume average particle size with a geometric standard deviation of about 1.51. About 1 part by weight of the encapsulated toner particles were mixed with about 99 parts by weight of 450 micron steel carrier

beads coated with about 0.4 percent by weight of a methyl terpolymer. In machine testing, this developer composition is found to provide excellent flat plate prints with or without the addition of a colloidal silica.

5

### Example XXIII

A sample of Xerox type 364 toner particles sold by the Xerox Corporation, Rochester, New York is employed 10 as a control. Copies of a standard test pattern are made with the toner. It is found by blocking tests that this toner material blocks at about 130 to 135° F. By comparison, it is found that the following toner compositions have a blocking temperature higher than 364 toner.

15

|    | Toner composition  | Blocking temperature, ° F. |
|----|--------------------|----------------------------|
|    | 364 toner -----    | 130-135                    |
|    | Example V -----    | 145-150                    |
|    | Example VII -----  | Greater than 180           |
| 20 | Example IX -----   | 155-160                    |
|    | Example XIII ----- | 150-155                    |
|    | Example XIV -----  | 150-155                    |
|    | Example XV -----   | 160                        |
| 25 | Example XVI -----  | 160                        |

The expression "developer composition" as employed herein is intended to include electroscopic toner material or combinations of toner material and carrier material.

30 Although specific materials and conditions are set forth in the foregoing examples, there are intended merely as illustrations of the present invention. Various other suitable toner resins, additives, colorants and other components, such as those listed above, may be substituted for those in the examples with similar results. Other materials 35 may also be added to the toner composition to synthesize, synergize, or otherwise improve the fusing properties or other desirable properties of the system.

Other modifications of the present invention will occur 40 to those skilled in the art upon a reading of the present disclosure. These are intended to be included within the scope of this invention.

What is claimed is:

1. An electrostatographic toner material comprising 45 finely-divided toner particles, said toner particles having a particle size range from about 0.5 to about 1,000 microns and a blocking temperature of at least about 100° F., said toner material comprising a colorant, said colorant comprising at least one member selected from the group consisting of pigments and dyes, an adhesive soft, 50 solid core material containing said colorant, and a shell material surrounding said core material.

2. The toner material as defined in claim 1 wherein 55 said core material is selected from the group consisting of polyesters, polyester based urethane polymers, epoxidized phenyl formaldehyde resin, docosyl acrylate/styrene copolymers, the polymeric reaction product of isopropylidenediphenoxypyropanol and adipic acid, and the polymeric reaction product of isopropylidenediphenoxypyropanol and sebacic acid.

3. The material as defined in claim 1 wherein said shell 60 is selected from the group consisting of polystyrenes, styrene-methacrylates, styrene-acrylates and polyethers.

4. The toner material as defined in claim 1 wherein 65 said core material has a viscosity at a shear rate of about 75 sec.<sup>-1</sup> of between about  $5 \times 10^4$  and about  $10^8$  poise at ambient temperature and a glass transition temperature below about 30° C. and wherein said shell material comprise an electrically insulating resin having a blocking 70 temperature of at least 100° F., a glass transition temperature above about 50° C., a modulus of elasticity of above about 100 p.s.i. and a compressive strength of above 500 p.s.i.

5. The toner material as defined in claim 1 further comprising 75 a powdered hydrophobic silica.

6. The toner material as defined in claim 1 wherein said core material is the polymeric reaction product of iso-propylidenediphenoxypyropanol and adipic acid.

7. The toner material as defined in claim 1 wherein said core material is the polymeric reaction product of iso-propylidenediphenoxypyropanol and sebacic acid.

8. The toner material as defined in claim 6 wherein said shell material is selected from the group consisting of polystyrenes, styrene-methacrylates, styrene-acrylates and polyethers.

9. The toner material as defined in claim 7 wherein the shell material is selected from the group consisting of polystyrenes, styrene-methacrylates, styrene-acrylates and polyethers.

## UNITED STATES PATENTS

|   |           |        |                       |          |
|---|-----------|--------|-----------------------|----------|
| 5 | 3,080,318 | 3/1963 | Claus -----           | 96—1 SD  |
|   | 3,645,911 | 2/1972 | Van Besauw et al. --- | 252—62.1 |
|   | 3,140,175 | 7/1964 | Kaprelian -----       | 252—62.1 |
|   | 3,318,697 | 5/1967 | Shrewsbury -----      | 96—1     |

J. TRAVIS BROWN, Primary Examiner

10 J. L. GOODROW, Assistant Examiner

U.S. Cl. X.R.

96—1 SD